

Patented Feb. 25, 1941

2,233,186

# UNITED STATES PATENT OFFICE

2,233,186  
WAX PAPER SHEET AND COATING  
THEREFOR

Randolph Spencer Soanes, Toronto, Ontario,  
Canada, assignor to Appleford Paper Products,  
Ltd., Hamilton, Ontario, Canada

No Drawing. Application July 11, 1938,  
Serial No. 218,636

1 Claim. (Cl. 91—68)

This invention relates to improvements in waxed paper sheets. More particularly it relates to improvements in wax coatings for paper sheets or the like and to the preparation of such coatings for application to sheets. Specifically, it relates to the provision of a transparent moisture proof heat sealable sheet of paper or the like which is suitable as a wrapping sheet wherever such a sheet is desired for use.

Heretofore heat sealable sheets have either been the low cost, low transparency wax paper sheets or the more expensive coated synthetic films. The latter type required in general that the coating be applied dissolved in suitable solvents, which solvents had to be evaporated off. Coatings of this latter type required expensive machinery not always possessed by the paper products manufacturer who specialized in hot melt coatings.

The low cost waxed sheets which are in widespread use are low in cost to manufacture as paraffin wax is commonly used as the coating material and as such coating can be applied as a hot melt by drawing a sheet to be coated through a vat containing the liquid coating but the sheets are low in transparency. To increase the transparency one common practice is to mix a low melt point ester gum with the paraffin. The ester gum increases the transparency but reduces the flexibility. While such ester gum paraffin coating can be applied as a hot melt in the same manner that paraffin is applied and increases substantially the transparency of the sheet it adds brittleness and the sheet does not heat seal satisfactorily.

Such coatings have heretofore been applied to thin tissue sheets of different kinds. Unfilled sulphite sheets and glassine paper sheets have been widely used. Glassine is more transparent and is grease resistant as compared with the unfilled sulphite sheet but the coating whether paraffin alone or the ester gum paraffin combination has a tendency to peel off the glassine base.

Furthermore, such a coated sheet does not possess the desired pliability but possesses rather an undesirable brittleness when folded or creased, which disadvantage is particularly unsatisfactory in a sheet designed to be moisture resistant.

My improved coated sheet possesses a high standard of pliability. The coating does not tend to break or crack upon folding or creasing the sheet. Where the base sheet is of substantial transparency the resulting transparency of the coated sheet is particularly high. My improved coated sheet possesses a high gloss and is odorless, colorless, and non-tacky. It is heat sealable and the seal produced is particularly secure. The sheet is moisture proof and is grease

proof, if a grease proof base sheet, such as glassine, is employed. My improved coating adheres securely to glassine and possesses high cohesive as well as adhesive characteristics. It is low in cost and the coating may be applied cheaply according to the hot melt method.

I have discovered that if a substance of a rubbery consistency, more particularly herein-after described, is added in a small quantity of from 2% to 5% of the total mixture to a mix of ester gum and paraffin that the coating will heat seal readily and form a particularly secure seal at the low temperatures of from 150° to 250° F., at which such sealing is commercially carried on and that such results may be obtained, even though the percentage of ester gum in the mix is increased substantially above that of the paraffin wax. The resulting coated sheet possesses all the desirable characteristics above enumerated and is particularly characterized by a high degree of flexibility without any tendency to break or crack along the line of fold or crease. My coating comprises:

|                                  | Per cent |
|----------------------------------|----------|
| Ester gum                        | 50 to 90 |
| Wax (paraffin)                   | 48 to 5  |
| Substance of rubbery consistency | 2 to 5   |

A formula which I have found very satisfactory is:

|                         | Parts  |
|-------------------------|--------|
| Ester gum approximately | 80     |
| Wax approximately       | 20     |
| Rubber approximately    | 2 to 3 |

As the ester gum constitutes the bulk of the mixture composition the melting point of such gum determines the temperature at which the coating may be applied as a hot melt. It is desirable that such temperature be maintained low because it is desirable to work at low temperatures and it is not desirable to bring the paraffin wax, which is the wax commonly used, to a high temperature or to maintain it at such high temperature for a protracted period because of the odor which it develops and which under certain conditions become permanent. Furthermore, the low melt point ester gums are more highly transparent than the high melt point ester gums, but the melting point should be sufficiently high so that the coating will not be tacky at room temperatures. I therefore prefer to employ a mixture of high and low melt point ester gums in the solution. A fifty-fifty mixture has been found suitable. Such a mixture possesses a high degree of transparency and is not tacky at room temperatures.

The ester gum increases the transparency of the coating substantially over that of a coating of paraffin wax alone. The ester gum, however, is not satisfactory for use alone as a coating be-

cause the coating produced by it is so brittle that it would break and flake off upon the bending of the sheet. Moreover, a sheet coated with ester gum alone or even a combination of ester 5 gum and paraffin will not heat seal satisfactorily, providing the ester gum is present in the coating mixture in such a proportion as to substantially increase the transparency, and to provide the desired transparency it is necessary to 10 use ester gum in the mixture in proportion of not less than 50% and preferably to an extent of approximately 80%.

The wax commonly used is paraffin wax and there is a variety of suitable melting point paraffins. Suitable animal, vegetable, or synthetic 15 waxes might be used but their price and the fact that they frequently develop rancid odors are deterrents to their employment in general. Paraffin waxes within the A. S. T. M. melting range of 20 125° to 150° F. are satisfactory. A paraffin wax within the 133° to 136° F. range has been found highly satisfactory. This paraffin wax may constitute 5% to 50% of the mixture. It is not ordinarily desirable to increase the amount of paraffin 25 over 50% as the transparency of the coating is thereby materially reduced. A coating consisting of substantially 50% paraffin and substantially 50% ester gum though possessing a fair standard of transparency will not satisfactorily 30 heat seal and has a low standard of flexibility but with the addition of even a small amount of the rubbery substance such a sheet heat seals satisfactorily and possesses the desired flexibility. A sheet coated entirely with paraffin will under 35 some circumstances heat seal satisfactorily but the transparency is low, however, a sheet of glassine coated with paraffin will not heat seal satisfactorily as there is a tendency for the coating to peel off. When the rubbery substance is 40 added however the heat seal is satisfactory and the coating is anchored securely to the base sheet.

Where the word "transparent" is used herein to describe the base sheet or the coated sheet it is not meant that the sheet is 100% transparent but 45 that a commercial degree of transparency is attained. It would characterize, for example, a sheet which might be termed semi-transparent or partially transparent.

Where the word "wax" is used herein to describe 50 this particular constituent of the composition paraffin wax is meant or some other suitable wax such as herein set forth.

The substance of a rubber consistency need be added in only a small percentage of from 2% to 55 5%. Such percentage may however be increased though the amounts specified have been found sufficient and it is not desirable to add such an amount of rubber as to increase the viscosity of the molten coating too high. On the other hand, 60 the rubbery substance may be reduced in amount below 2 parts for 100 parts of mix. Even one per cent or less of rubber in the mixture is helpful. This rubbery substance may be in the form of crepe rubber or smoked rubber sheets. Synthetic 65 rubber or a substance of a similar rubbery consistency which might not even be termed a true synthetic rubber may be used. An example of a synthetic material of a rubbery consistency which I have found suitable is the polymer of iso-butylene (2 methyl propylene) sold under the trade 70 name of Vistanex-Medium.

This substance of a rubbery consistency must possess the capacity to go into solution with the other ingredients, such as paraffin and ester gum. When I use the phrase "going into solution" I mean that this is apparently the result. Some 5 authorities might, however, term it a dispersion so finely divided and distributed as not to be visible. At least it is a solution to the extent that it does not separate out and appears to be 10 in solution.

In the preparation of my coating composition or mixture I may incorporate as by means of a rubber mill or otherwise one part of the substance of a rubbery consistency from with one to five parts of wax or alternative ester gum. I have found 15 that two parts of wax worked in with one part of the substance of a rubbery consistency is very satisfactory. This mixture of the rubbery substance and wax is then melted together with the necessary wax and ester gum to complete the 20 formula. This operation may be conveniently carried out in the actual tanks of the coating machine. The melt is stirred until homogeneous and the rubbery substance goes into solution as described. When the term "substance of a rubbery consistency" or "rubbery substance" is used herein it is intended to include synthetic substances such as above set forth as well as the natural rubber. 25

A simplified method of incorporating the rubbery substance in the solution and one which I have found preferable is to gradually add small fragments of pale crepe rubber sheets to a solution of molten paraffin heated to approximately 20° C. above its melt point while subjecting 30 said solution during such incorporation to violent stirring and agitation. Such temperature and agitation should be continued for the time required to bring the rubbery substance completely into solution, which should be accomplished within twelve hours or less. The ester gum constituents may then be stirred into the solution and thoroughly incorporated therein. 40

The sheet material to be coated is then run through the machine in the ordinary manner of 45 application of a hot melt coating. In one preferred form of the invention the base sheet is a plasticized glassine. A fine tissue sheet, such as an unfilled sulphite sheet, may be used which would produce a strong sheet though less transparent than the coated glassine sheet. The resulting coated sheet possesses high transparency. For example, if glassine is employed the coated sheet possesses a substantially higher degree of transparency than the base glassine sheet. The 55 coated sheet hot seals splendidly, is non-tacky, possesses a fine gloss, and is substantially transparent and moisture resistant.

One or both sides of the base sheet may be 60 coated. The transparency will be increased by coating both sides and such is generally the approved procedure. If desired, the sheet may be printed before coated.

What I claim: 65  
A sheet of the character described comprising a cellulose base sheet having a surface portion coated with a composition consisting of approximately eighty parts ester gum, approximately twenty parts paraffin wax, and approximately two to three parts of rubber. 70

RANDOLPH SPENCER SOANES.